

## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## PROCESS OF TREATING CELLULOSE FIBER AND PRODUCT OF SAME

No Drawing.

Application filed June 2, 1927. Serial No. 196,135.

In the various industries in which cellulose is employed as a raw material, it has heretofore been the practice to treat the cellulose in the form of fiber of substantially natural or original size. Thus, in the preparation of cellulose derivatives such as xanthate, acetate, nitrate, etc., cotton fiber or fiber liberated from wood is treated substantially in the same size as it is found in nature.

10 Owing to the widely varying sizes of cellulose fibers as they occur in nature, it is sometimes inefficient to process cellulose fiber in its natural condition. For instance, in manufacturing rayon by the viscose-rayon process, it has been the practice to treat cellulose fiber with caustic soda solution, and then to age the treated fiber to effect its depolymerization for xanthation. In order to effect a substantially complete xanthation 20 of the fiber, it is necessary to effect a thorough depolymerization of substantially all the fiber. Inasmuch as the longer and thicker fibers require a longer aging period than the smaller fibers, a long aging period is necessary to effect the desired complete depolymerization; and, in such case, the small fibers are depolymerized more than the larger ones, frequently being over-depolymerized. The aged fiber is thus made up of fibers depolymerized to widely varying degrees.

In accordance with the present invention, cellulose fiber as it is obtained from nature is materially reduced in size prior to use or to chemical treatment, thereby producing a raw material of much greater chemical reactivity and which hence reacts much more rapidly and completely when treated with chemical reagents. Such size reduction is particularly advantageous in the viscose-rayon process, as I have found that by materially reducing the fiber in size prior to processing, the aging period may be greatly reduced, if not entirely eliminated, and a substantially uniformly depolymerized product obtained. I have also found that by so doing I am enabled to carry out the other steps of the viscose-rayon process more rapidly and effectively than heretofore. Thus, the reduced fiber can be uniformly permeated with caustic soda solution more rapidly, and xanthates the soda

cellulose thus produced more readily and completely. Reduction of the original fiber to materially smaller size may be accomplished expediently by beating, but this operation need not be carried out under conditions to effect its hydration, as is customary in papermaking.

A process such as described may be applied to great advantage in treating cellulose fiber of high average fiber length,—for example, 60 the long fiber portion of a high alpha cellulose wood fiber. Such long fiber portion is notably free from specks, colloidal coloring material, resin, ash, and other contaminations, and is hence eminently suitable for derivative preparation, but heretofore the use of such fiber involved an especially long and troublesome aging period.

A better understanding of the process of the present invention may be obtained from the following more complete description thereof, which relates to viscose-rayon processing of a high alpha-cellulose wood fiber, which for convenience of designation will hereinafter be termed alpha wood fiber. It is to be understood, however, that my invention may be applied to the preparation of other derivatives and to other wood fiber, such as sulphite fiber, or to cellulose fiber of other derivations, such as cotton fiber. An alpha wood fiber such as I employ may be prepared by the process disclosed in application, Serial No. 716,154, filed May 27, 1924, by Milton O. Schur and myself. In accordance with that process, chemical wood fiber, such as sulphite pulp, is subjected to a series of chemical treatments, including an initial treatment with chlorine water, followed by digestion in an alkaline liquor and a final bleaching treatment, which effect a removal of non-alpha cellulose components therefrom to produce a white fiber of high alpha cellulose content and especially low in impurities such as lignin, resins, pentosans, and oxy-celluloses. More particularly, as described in that application for patent, the unbleached sulphite pulp is initially treated for about thirty minutes as a 10% stock suspension with 0.3% to 0.6% of chlorine, or with 1% to 2% of hypochlorite bleach, based on the

weight of dry pulp. The pulp is then washed and digested from two to six hours at elevated temperature in an alkaline liquor of a strength of 0.1% to 0.5% caustic soda, or from 1% to 5% caustic soda, based on dry pulp. The pulp is again washed and then treated in the form of a 10% suspension at a temperature of about 80° F. and for from six to eight hours with 2% to 4% of hypochlorite bleach, based on dry pulp, whereupon the bleached product is thoroughly washed and treated with suitable antichlor, such as calcium bisulphite, to neutralize any bleach that may remain in the product.

If desired, the long fiber portion, which yields rayon of the highest quality, may be selected from the rest of the fiber and then treated by my process, but obviously all the fiber may be so treated. In accordance with my process, the fiber is materially reduced in size, as by beating, but this operation need effect only a shortening or cutting of the fiber, as I am not especially interested in effecting its hydration, as is desired by the papermaker, nor in producing paper having good physical characteristics. Thus, beating may even be effected in a jordan or in a Hollander in which the beater roll is provided with very sharp blades set to clear the bed-plate only slightly, and may even be carried out at elevated temperature,—this being undesirable in usual papermaking procedure, as elevated temperature tends to decrease the hydratability of cellulose fiber. The beating is preferably continued until the original fiber has been considerably reduced in average fiber length and width. Thus, a typical alpha wood fiber having an average fiber length of, say, from 0.7 to 1.3 mm. may be beaten until its average fiber length has been reduced to below 0.2 mm.

The shortened fiber may then be run off into the so-called drier sheet usually supplied to rayon manufacturers, but preferably, however, it is run off into waterleaf paper, as described in my application, Serial No. 194,506, filed May 26, 1927, wherein the advantages of processing fiber of short length in paper form are disclosed. The shortened fiber is of notably lower viscosity than the original fiber, this quality apparently denoting depolymerization. Thus, the shortened fiber requires little, if any, aging prior to xanthation, whereas the original fiber requires considerable aging to acquire the same viscosity and reactivity.

The viscose-rayon processing of such reduced fiber may be carried out substantially as follows: the drier sheet or paper composed of the reduced fiber is saturated with caustic soda solution, as usual, to effect a conversion of the fiber into soda cellulose. Inasmuch as the fibers are small, they are rapidly and uniformly permeated throughout with the solution, and hence become uniformly con-

verted into soda cellulose. After the excess solution has been removed from the drier sheet or paper, it is shredded into crumby flocks, which may be xanthated with little, if any, aging. The xanthated fiber dissolves quite readily in caustic soda solution to produce a xanthate solution suitable for spinning and containing little unxanthated fiber. By the process of the present invention, I am thus enabled to eliminate or, in any event, to shorten considerably the usual aging period of from 48 to 120 hours. I am also enabled to obtain a substantially uniformly depolymerized fiber for xanthation.

The reduction of the fiber may, if desired, be continued by beating or other mechanical treatment until it has been reduced to a pulverulent condition and can no longer be sheeted but must be handled and treated in bulk form as in the form of bulk powder or compressed cakes, or in the form of a suspension in water or other liquid vehicle. Inasmuch as cellulose in such condition has a very large aggregate surface, it is exceedingly reactive and may hence be converted into cellulose xanthate or other cellulose derivatives very rapidly and completely. Furthermore, it is adapted for other uses requiring substantially pure cellulose in non-fibrous condition. Thus, when prepared from cotton fiber or from a wood fiber such as alpha fiber, it consists essentially of alpha cellulose only, and may hence serve as a raw material not only for the preparation of substantially pure cellulose derivatives but also as a filler in products requiring non-fibrous cellulose substantially free of non-alpha cellulose components.

When it is desired to produce a very finely divided powder, say, one substantially all of which passes through a 100-mesh screen, it is necessary to pulverize or to complete pulverization in apparatus other than a beater. In such case, pulverization may, for instance, be effected by passing the dry fiber, partly reduced by beating if desired, through a suitable ball or roller mill, which serves to pound or grind the fibers into a finely divided powder.

The powder may be separated from residual coarse particles or fiber, as by air flotation, and the coarse particles or fiber returned to the mill for regrinding. If it is desired to pulverize the fiber by a wet process, it is preferable either to convert the fiber to a non-hydratable condition or to pulverize in a non-hydrating wetting medium, as hydration of the fiber appears to hinder its pulverization. Thus, the fiber may be mercerized or converted into regenerated cellulose fiber, in which case pulverization may be performed in the presence of water, as mercerized or regenerated cellulose fiber is non-hydratable. Or the hydratable fiber may be pulverized in a wetting medium such

as alcohol or benzol, which is of a non-hydrating character.

In some of the appended claims, I speak of "individualized cellulose fibers," by which expression I mean fibers in a separate or individual condition, as obtains in the case of wood pulps or cotton, as distinguished from the condition of the fiber in wood, nut shells, or the like, where they are bound together as a rigid mass of cementitious material. While it is easy to grind a rigid mass such as wood or nut shells into a powder, nevertheless the treatment of the powder with chemical solutions such as those of alkali to dissolve out non-alpha cellulose components is accompanied by a vastly greater loss of alpha cellulose than is the case when the fibers are first liberated from the cementitious material and then mechanically reduced as separated or individualized fibers.

By the term "cellulose fiber" as employed herein and in the appended claims, I mean not only a substantially pure form of cellulose such as cotton fiber or a refined wood fiber composed essentially of alpha cellulose, but also the usual commercial wood fibers, e. g., sulphite fiber, which, in addition to alpha cellulose, contain a certain small proportion of non-alpha cellulose components such as pentosans, beta and gamma celluloses, oxycelluloses, and the like, but which have an alpha cellulose content materially above 60%.

In carrying out the shortening or reduction of the fiber as in a powder engine or in a ball mill, as hereinbefore described, it is clear that the fiber is in the form of a mass in which the fiber units are in random arrangement. In other words, the process of my invention does not require that the fiber used as a raw material be subjected to special manipulation designed to produce a particular fiber arrangement or formation, for instance, parallelism of fiber units, such as is brought about when cutting fibers are subjected to the action of carding machines.

I do not herein claim specifically the subject matter of application, Serial No. 122,271, filed July 13, 1926, which discloses the beating or hydration of cellulose fiber prior to viscose-rayon processing, or the subject matter of application, Serial No. 194,506, filed May 26, 1927, which discloses the advantages of using waterleaf paper composed of reduced fiber. Nor do I herein claim the subject matter of its continuation application Serial No. 97,998, filed March 27, 1926, by Milton O. Schur, Royal H. Rasch and myself, wherein the advantages of beating cellulose fiber prior to nitration are disclosed, or the subject matter of its continuation application, Serial No. 140,674, filed October 9, 1926.

What I claim is:

1. A process which comprises beating cellulose fiber below an average fiber length of

0.2 mm. while maintaining it substantially free from chemicals, and then converting the reduced fiber into a cellulose derivative.

2. A process which comprises beating cellulose fiber until its average fiber length has been shortened to below 0.2 mm. while maintaining it substantially free from chemicals, and then converting such beaten fiber into cellulose xanthate.

3. A process which comprises materially reducing cellulose fiber in size while maintaining it substantially free from chemicals, then treating such reduced fiber with caustic soda solution, aging the treated fiber for only a short period, and then xanthating the aged fiber.

4. A step which comprises pulverizing cellulose fiber in the presence of a non-hydrating wetting medium.

5. A product consisting of mechanically pulverized wood substantially free from non-alpha cellulose components.

6. A process which comprises converting a product consisting of mechanically pulverized wood fiber substantially free of non-alpha wood components into cellulose derivative.

In testimony whereof I have affixed my signature.

GEORGE A. RICHTER. 95

100

105

110

115

120

125

130